

## UNITED STATES PATENT OFFICE

2,395,475

## BENEFICIATION OF BERYLLIUM ORES

Harold L. Gibbs and Henry D. Snedden, Salt Lake City, Utah, assignors to the Government of the United States, as represented by the Secretary of the Department of Interior

No Drawing. Application March 2, 1945,  
Serial No. 580,578

4 Claims. (Cl. 209—166)

(Granted under the act of March 3, 1883, as  
amended April 30, 1928; 370 O. G. 757)

The invention described herein may be manufactured and used by or for the Government of the United States for governmental purposes without the payment to us of any royalty thereon in accordance with the provisions of the act of April 30, 1928 (Ch. 460, 45 Stat. L. 467).

This invention relates to the beneficiation of beryllium ores and has for its object the production of a high grade beryllium ore concentrate from low grade beryllium deposits. Another object is the provision of a process whereby relatively coarse beryllium ore having an average particle size as large as plus 100-mesh or larger, can be beneficiated through a selective mineral-filming technique.

The foregoing and other objects hereinafter apparent are accomplished in accordance with this invention wherein a beryllium ore is beneficiated by subjecting such an ore to a mineral-concentrating treatment involving selective filming under acidic conditions of a desired constituent in the presence of a soluble fluoride, a long-chain fatty acid and a long-chain alkyl amine salt. It has been found that beryllium ores can be beneficiated to produce high grade concentrates even though relatively coarse beryllium ore be employed having an average particle size at least as large as plus 100-mesh, for example, between 20 and 100-mesh as determined by standard Tyler screens, when the mineral-concentrating treatment is carried out in the presence of a long-chain alkyl amine salt, such as for example lauryl amine hydrochloride.

Suitable beryllium ores for employment in accordance with this invention include ores containing beryl, chrysoberyl and other beryllium minerals containing gangues of widely varying composition including such constituents for example as mica, quartz, apatite, iron compounds, pegmatite, feldspar, tourmaline and other gangue materials normally associated with beryllium minerals. The ores may be treated in a wide range of particle size in accordance with this invention, such as for example in minus 10-mesh to minus 800-mesh, and we have found that our

invention provides a very high recovery in the larger particle sizes at least as large as plus 100-mesh not hitherto successfully concentrated.

It has been found that the presence of metallic iron or iron compounds exerts a detrimental influence on the beneficiation of beryllium ores by mineral filming techniques such as for example agglomerative tabling or froth flotation, and therefore we prefer to subject the selected ore to an iron removal treatment, preferably after initial grinding. For example, we may remove the so-called "grinding iron" introduced during grinding in iron ball mill equipment together with magnetic iron compounds which may be present in the ore, by subjecting the comminuted ore to wet magnetic separation. This is accomplished in the usual way by passing the ore pulp over a suitable magnet such as for example an electromagnet. A preferred iron removal treatment, which may be employed alone or in conjunction with magnetic separation, is the treatment of the comminuted ore pulp with a strong mineral acid such as for example hydrochloric acid, nitric acid, hydrofluoric acid, sulfuric acid, and preferably a mixture of a soluble fluoride with sulfuric acid. After the acid treatment, the soluble iron compounds produced are removed together with slimes by washing the ore sands with a large excess of water. The foregoing acid treatment in conjunction with a soluble fluoride constitutes a preferred conditioning treatment or pretreatment in accordance with this invention and not only serves the function of removing iron, but also renders the desired beryllium minerals peculiarly receptive to selective filming with the reagents hereinafter to be described.

Following the pre-treatment or conditioning, the beryllium ore can be concentrated by agglomerative tabling employing preferably oleic acid, No. 1 or similar fuel oil, and a soluble salt of a long-chain alkyl amine. This is accomplished in the usual manner by passing an aqueous pulp of the ore and reagents across a reciprocating table such as for example a Wilfley table provided with a cross wash of water. The

beryllium agglomerates are carried over the side of the table and the gangue particles proceed over the end of the table. Flotation, involving agitating and aerating the ore pulp with reagents and separating the mineral-bearing froth, is a preferred concentrating treatment involving selective filming in our invention.

Regardless of the mineral concentrating treatment employed, it has been found that a desirable recovery can be made when the treatment is carried out in the presence of a long-chain alkyl amine salt. Suitable long-chain alkyl amine salts are the formates, acetates, sulfates, and preferably the hydrochlorides of aliphatic amines having from 8 to 18 carbon atoms in the alkyl radical. The commercial mixture of the long-chain aliphatic amine hydrochlorides derived from the fatty acids present in coconut oil, sold under the trade name "D. P. 243" and the mixture believed to contain largely lauryl amine hydrochloride sold under the trade name "E. P. 487," have been found to be especially suitable long-chain alkyl amine salts for employment in accordance with this invention although salts of long-chain aliphatic amines derived from or corresponding to the fatty acids produced from other vegetable, animal, marine, and synthetic sources can be employed. Generally, the long-chain alkyl amine salt is employed in proportions of from 0.1 to 5 pounds of the commercially sold mixture per ton of ore and is preferably employed in the somewhat more restricted proportions of between 0.3 and 3.5 pounds of the commercial mixture per ton of ore. Greater or lesser amounts can also be used.

Suitable soluble fluorides for employment in the conditioning or pre-treatment step and also in the flotation or agglomeration stage, are the alkali metal fluorides including sodium and potassium fluoride, and other compounds yielding a fluoride ion under acidic aqueous conditions, such as for example, sodium silicofluoride. Generally sodium fluoride or other soluble fluoride is employed in proportions of from 0.2 to 10 pounds of soluble fluoride per ton of ore and preferably within the more restricted range of between 2 and 5 pounds of soluble fluoride per ton of ore being treated. Hydrofluoric acid is a very desirable soluble fluoride and in addition provides the necessary acidic conditions for carrying out this invention, but in general, because of handling difficulties, we prefer to employ sodium fluoride in conjunction with sulfuric acid.

Both the pre-treatment or conditioning step and the flotation or tabling step in our invention are carried out under acidic conditions, by which is meant under a pulp acidity at least as acid as pH 6.9. Generally, the pH of the pulp during conditioning and tabling or flotation is maintained within a pH between about pH 1.5 and pH 6.5, while preferably the acidity is maintained between pH 2 and pH 6.

The selective filming treatment of this invention whether it be agglomerative tabling or flotation, is carried out in the presence of a long-chain fatty acid having from 8 to 18 carbon atoms, as a mineral-filming reagent. Representative long-chain fatty acids are stearic acid, palmitic acid, lauric acid and preferably oleic acid. Other suitable fatty acids include the mixture of fatty acids derived from the oils of coconut, tallow, sardine, menhaden, whale, cotton seed, peanut, and similar vegetable, animal and marine oils. The fatty acid is admixed with the pre-treated ore pulp in controlled amounts sufficient to float the desired

constituent, in flotation or sufficient to agglomerate the desired constituent in the case of the agglomerative tabling. A suitable amount of oleic or other fatty acid to employ is from 0.2 to 10 pounds of long-chain fatty acid per ton of ore undergoing treatment. Since the fatty acid probably exists largely in the free state in our acidic ore pulp, it is desirable to introduce it in the form of an aqueous emulsion to provide for its better dispersion in the ore pulp. A suitable emulsifying agent comprises the ammonium salt of lauryl diethylene glycol sulfate sold under the trade name "Emulsol X-1," although other emulsifying agents can be used. It is preferably employed in amounts of from 0.1 to 2.0 pounds per ton of ore undergoing treatment.

In carrying out our invention, it is often desirable to subject the ore pulp to a preliminary flotation employing very restricted proportions of reagents to selectively remove the mica contained in the ore. Likewise, various other mineral beneficiating treatments known to the art can be employed in conjunction with our process.

The following illustrative examples show how the invention may be carried out but it is not restricted thereto. Parts and percentage compositions are by weight unless otherwise designated.

#### DESCRIPTION OF ORES TESTED

Much of the test work was done on an 800-pound sample of ore from the Wisdom Ranch, Larimer County, Colorado. This sample assayed 0.94 percent BeO and consisted of beryl and chrysoberyl associated with oligoclase feldspar, quartz, muscovite, and garnet. The bulk of the beryl occurs in plus 10-mesh sizes; however, enough beryl and chrysoberyl occur finely intergrown at contact areas with gangue rock to necessitate fine grinding of the ore for optimum beryllium recovery.

Other test work was done on two samples of low-grade beryl ore from the Mica Mountain District, Latah County, Idaho. One of these samples assayed 0.39 percent BeO and represented the minus  $\frac{1}{2}$ -inch rejects from a screening and hand sorting operation. The lower grade sample assayed only 0.17 percent BeO. Mineralization of both samples was similar. Principal minerals were beryl, muscovite, feldspars, quartz, tourmaline, magnetite, and apatite. Beryl occurred as fragments ranging in size from about  $\frac{1}{4}$ -inch to 100-mesh; most of the beryl was liberated by grinding the ore through 65-mesh.

Commercial grade products, approximately 10 percent BeO, were made from all three ores. Several products obtained assayed between 12 and 13 percent BeO which is approximately the BeO content of pure beryl mineral.

#### TEST PROCEDURES

##### COARSE GRAVITY

Where part of the beryl in an ore occurred in coarse crystals, it was partially concentrated by gravity at coarse sizes by sink-and-float methods. Standard laboratory procedures were used and both galena suspensions and heavy liquids were found to be satisfactory. Test results indicate that the method would be of most value when used to reject coarse waste rock with a minimum of crushing rather than as a complete concentration process used to make finished beryl products.

## AGGLOMERATION TABLING

Beryl was concentrated at intermediate sizes using agglomeration tabling. Commercial grade concentrates were made. The beryl was not readily agglomerated until the ore had been given a special acid-fluoride conditioning treatment as described later under flotation (Step 3). Following this conditioning treatment, the ore was washed, agglomerated with oleic acid and No. 1 fuel oil, and tabled.

## FLOTATION

Preliminary flotation tests following published flotation procedures and reagent combinations were not satisfactory. A successful procedure was finally developed that involved flotation of deslimed sands after a special conditioning treatment which is described as follows:

## BASIC PROCEDURE FOR BERYL FLOTATION

1. The ore is roll crushed dry to approximately 10-mesh and, with small additions of NaF (0.2 pound per ton), is stage ground wet through 100-mesh in an iron ball mill.

2. Minus 100-mesh ore is deslimed by decantation and grinding iron is removed from sands by wet magnetic separation.

3. Sands are conditioned for approximately 30 minutes in a laboratory flotation machine (a mechanical agitation flotation machine having a glass cell and rubber coated metal parts), at a pH of 2.0 to 2.5 with NaF (3 to 6 pounds per ton) and H<sub>2</sub>SO<sub>4</sub> (7 to 15 pounds per ton) filtered and washed.

4. Filter cake is repulped in flotation machine with fresh water, NaF (0.2 pound per ton), H<sub>2</sub>SO<sub>4</sub> (for a pH of 6.0 to 6.9), conditioned for 5 minutes with a water emulsion of oleic acid stabilized with Emulsol X-1 and the beryl is floated.

Satisfactory recovery of beryl was obtained in a high-grade product when HF and HCl were substituted for NaF and H<sub>2</sub>SO<sub>4</sub> in conditioning step 3 of basic procedure. Substitution of CaF<sub>2</sub> for NaF was not satisfactory as the calcium ion consumed oleic acid and probably activated gangue minerals. Small additions of fluoride to grinding and beryl flotation circuits were beneficial but not essential. Using the above procedure, flotation of minus 100-mesh beryl was rapid and the products were clean, but flotation of plus 100-mesh beryl was slow and the products were not clean. Washing sands by decantation was as effective as filtering and washing on the filter.

The following modifications were made on the basic procedure to improve separation of beryl from certain minerals.

A. Dry beryl concentrates were treated on a high intensity, ring type, magnetic separator to remove garnet and other magnetic minerals. In addition to floating beryl, oleic acid also collected minerals such as garnet, tourmaline, and biotite. No attempt was made to selectively float beryl from these minerals as the separation was readily made magnetically and the quantity of such impurities was small.

B. In general, mica was effectively depressed when using the previously outlined basic procedure for beryl flotation. However, where the mica to beryl ratio of low-grade ores was high, it was advantageous to remove mica before the beryl was floated. It was possible to float mica at coarse sizes, which would aid in reducing grinding costs, and, from suitable ores, clean commercial grade mica by-products could be

made. Mica was selectively floated using an alkyl amine salt such as D. P. 243 or E. P. 487 as collector and frother. The mica could be floated either from an acid circuit prior to the acid-fluoride conditioning step or from the acid-fluoride circuit itself. The amine salt used to float mica was also a collector for chrysoberyl and if this mineral were present in the ore, the mica float had to be made very carefully or some chrysoberyl was lost in the mica concentrate. Beryl was activated by the amine salt; after activation, coarse beryl was more easily floated with fatty acid. The activation of coarse beryl by an amine salt in the acid-fluoride conditioner was effective even though a mica float was not actually made. When a separate mica float was not made, the amine salt caused some mica to float with the beryl, but concentrates assaying plus 10 percent BeO were still readily obtained.

C. Apatite and beryl were separated by selective flotation. Apatite floats more readily than beryl and by careful additions of oleic acid was floated ahead of beryl to make a separate rougher concentrate. If this separate rougher concentrate was not made, the selective flotation of apatite from beryl was difficult although sometimes still possible. The apatite rougher concentrate containing some beryl was conditioned with NaOH at a pH of 11.5 filtered, washed, repulped with water, and the apatite selectively floated at a pH of 8.4 using small additions of X-1. Any apatite remaining in the beryl concentrate could be leached out with dilute acid.

D. The substitution of caustic for acid-fluoride in the conditioning stage was partially successful provided a pebble mill was used to grind the ore. Results were inferior to those obtained with acid-fluoride and no separation of beryl could be made if the ore had been ground in an iron ball mill.

Results of typical tests, making use of the concentration procedures just discussed, are given for three western beryl ores.

## EXAMPLES NOS. 1 AND 2.—WISDOM BERYL

The first successful flotation tests were run while employing special grinding procedures. The major object was to reduce iron contamination during grinding. In one test the ore was roll crushed dry through 20-mesh; after removing the metallic iron with a wet magnetic separator, the minus 20-mesh product was stage ground wet through 100-mesh in a pebble mill and deslimed. In another test the ore was roll crushed dry through 10-mesh and stage ground dry through 100-mesh in an iron ball mill; the grinding iron was removed on a magnetic separator, and the ore pulped with water and deslimed. In both tests concentration procedures were the same; mica and beryl were selectively floated and the dried beryl concentrates were treated on high intensity magnetic separator to remove garnet.

Reagent consumptions and test results are tabulated for both tests in Tables 1 and 1A.

TABLE 1.—REAGENT CONSUMPTION IN POUNDS PER TON OF ORE

| 70                     | HF 45% | HCl | D. P. 243 | Oleic acid | X-1 |
|------------------------|--------|-----|-----------|------------|-----|
| Pebble mill grind..... | 2.0    | 4.8 | 0.06      | 2.0        | 0.4 |
| Ball mill grind.....   | 2.0    | 4.8 | 0.23      | 1.0        | 0.2 |

TABLE 1A

| Test products             | Weight, percent |           | Assay, percent BeO |           | Distrib. percent BeO |           |
|---------------------------|-----------------|-----------|--------------------|-----------|----------------------|-----------|
|                           | Pebble mill     | Ball mill | Pebble mill        | Ball mill | Pebble mill          | Ball mill |
| No. 1 beryl concn.        | 6.0             | 7.1       | 10.25              | 10.45     | 66.1                 | 71.8      |
| No. 2 beryl concn.        | 2.0             | 1.6       | 5.75               | 0.70      | 12.4                 | 1.0       |
| Rougher flotation tailing | 52.5            | 47.2      | 0.01               | 0.01      | 0.5                  | 0.5       |
| Mica concentrate          | 18.0            | 25.1      | 0.23               | 0.53      | 4.4                  | 12.9      |
| Slimes                    | 21.0            | 18.6      | 0.73               | 0.75      | 16.4                 | 13.6      |
| Magnetic product          | 0.5             | 0.4       | 0.34               | 0.50      | 0.2                  | 0.2       |
| Total head                | 100.0           | 100.0     | 0.93               | 1.03      | 100.0                | 100.0     |

By flotation of minus 100-mesh ore, 66.1 and 71.8 percent of the beryllium were concentrated in products assaying 10.25 and 10.45 percent BeO, respectively. Loss of chrysoberyl in mica concentrate was roughly proportional to the weight floated and the amount of D. F. 243 used. Loss of BeO in the slime fraction was 13 to 16 percent as compared with 20 to 22 percent when conventional wet ball mill grinding procedures were employed.

#### EXAMPLE NO. 3.—WISDOM BERYL

A locked roughing test was run, in six cycles, to determine the effect of returning middlings to the flotation circuit. Each sample was stage ground wet to minus 100-mesh in a laboratory ball mill. In this test the basic flotation procedure was employed except that the second rougher concentrate or middling from each flotation stage was re-treated with new ore in the next flotation stage. All concentrates and the small amount of final middling were combined and cleaned by flotation, using the same procedure as in the rougher flotation circuit. Cleaner flotation concentrate was dried and treated on a magnetic separator to remove garnet. Reagent consumptions and test results tabulated in Tables 2 and 2A.

TABLE 2.—REAGENT CONSUMPTION IN POUNDS PER TON OF ORE

| H <sub>2</sub> SO <sub>4</sub> | NaF | Oleic acid | X-1  |
|--------------------------------|-----|------------|------|
| 15.4                           | 7.4 | 1.47       | 0.29 |

TABLE 2A

|                            | Weight percent | BeO, percent |              |
|----------------------------|----------------|--------------|--------------|
|                            |                | Assay        | Distribution |
| Beryl concentrate          | 8.10           | 11.3         | 76.0         |
| Cleaner flotation middling | 1.10           | 1.98         | 1.8          |
| Cleaner flotation tailing  | 2.97           | 0.07         | 0.2          |
| Rougher flotation tailing  | 62.61          | 0.013        | 0.7          |
| Slimes                     | 23.51          | 1.06         | 20.7         |
| Magnetic product           | 1.71           | 0.43         | 0.6          |
| Total head                 | 100.00         | 1.20         | 100.0        |

By flotation of minus 100-mesh ore, 76 percent of the BeO was recovered in a product assaying 11.3 percent BeO. Mica was effectively depressed and no special mica separation was needed. Test results indicate that the process can be operated on a continuous basis and middlings re-treated to recover the beryl they contain. It should be noted that loss of BeO in slime is 20.7 percent as compared with only 16.4 and 13.6 percent when special grinding procedures, previously described, were used.

#### EXAMPLE NO. 4.—WISDOM BERYL

In an attempt to reduce loss of beryl in slimes, a test was run in which coarse ore was treated by sink-and-float and hand sorting while fine ore was treated by flotation. Ore, as received, was screened on 1-inch, ½-inch, 3-mesh, and 20-mesh screens. The minus 20-mesh material, consisting largely of top soil and roots with very little beryl, was discarded without treatment. The plus 3-mesh portions were treated separately by sink-and-float using galena suspensions of 2.60 and 2.66 specific gravities to reject coarse feldspar and quartz, respectively. Sink products were hand sorted to remove free beryl crystals. Hand-sorted rejects were combined with the original minus 3 plus 20-mesh material and the composite was stage ground to minus 100-mesh and floated to recover beryl. Dry beryl flotation concentrate was treated in the high intensity magnetic separator to remove garnet.

Reagent consumptions and test results are tabulated in Tables 3 and 3A.

TABLE 3.—REAGENT CONSUMPTION IN POUNDS PER TON

|                | H <sub>2</sub> SO <sub>4</sub> | NaF | Oleic acid | X-1  |
|----------------|--------------------------------|-----|------------|------|
| Flotation feed | 22.0                           | 8.0 | 2.0        | 0.5  |
| Original ore   | 8.4                            | 3.3 | 0.8        | 0.18 |

TABLE 3A

|                                       | Weight percent | BeO, percent |              |
|---------------------------------------|----------------|--------------|--------------|
|                                       |                | Assayed      | Distribution |
| Sorted plus 1-inch beryl              | 0.32           | 11.9         | 4.3          |
| Sorted minus 1 plus ½-inch beryl      | 1.99           | 12.6         | 28.2         |
| Sorted minus ½-inch plus 3-mesh beryl | 1.20           | 12.45        | 16.7         |
| Beryl flotation concentrate           | 2.69           | 9.52         | 28.7         |
| Slimes                                | 10.43          | 1.00         | 11.7         |
| Quartz "float" at 2.60 sp. gravity    | 12.32          | 0.11         | 1.5          |
| Feldspar "float" at 2.60 sp. gravity  | 33.54          | 0.05         | 2.0          |
| Rougher flotation tailing             | 24.65          | 0.11         | 3.0          |
| Original minus 20-mesh discard        | 12.30          | 0.26         | 3.6          |
| Magnetic product                      | 0.56           | 0.61         | 0.3          |
| Total head                            | 100.00         | 0.89         | 100.0        |
| Composite beryl concentrate           | 6.20           | 11.2         | 77.9         |

Using a combination method, treating coarse ore by sink-and-float and hand sorting and fine ore by flotation, 77.9 percent of the BeO was concentrated in a product assaying 11.2 percent BeO. Principal beryl loss is still in the slime fraction. However, this loss is lower than in tests in which all of the ore was ground to flotation sizes.

#### EXAMPLE NO. 5.—WISDOM BERYL

Treatment of coarse sizes of ore by agglomeration tabling also was tried to reduce slime losses. A sample of ore was roll crushed dry through 20-mesh and screened on 35-mesh and 65-mesh screens. The plus 65-mesh sizes were conditioned with acid-fluoride, as in step 3 of the basic flotation procedure, beryl was agglomerated with oleic acid and No. 1 fuel oil and the ore tabled. Minus 65-mesh ore was ground through 100-mesh and the beryl was floated. Mica that contaminated all beryl concentrates was removed by elutriation. Dry beryl concentrates were treated on a high intensity magnetic separator to remove garnet.

Reagent consumptions and test results are tabulated in Tables 4 and 4A.

TABLE 4.—REAGENT CONSUMPTION IN POUNDS PER TON OF ORE

|                       | H <sub>2</sub> SO <sub>4</sub> | NaF | Oleic acid | X-1  | No. 1 fuel oil |    |
|-----------------------|--------------------------------|-----|------------|------|----------------|----|
| Agglomeration tabling | 1.8                            | 0.4 | 0.28       |      | 0.23           | 10 |
| Flotation             | 2.3                            | 0.7 | 0.25       | 0.05 |                |    |
| Total                 | 4.1                            | 1.1 | 0.53       | 0.05 | 0.23           |    |

TABLE 4A

|                             | Weight, percent | BeO, percent |              | 20 |
|-----------------------------|-----------------|--------------|--------------|----|
|                             |                 | Assay        | Distribution |    |
| Agglomerate concentrate     | 5.46            | 9.5          | 52.5         |    |
| Flotation concentrate       | 1.18            | 10.2         | 11.1         |    |
| Table rejects               | 60.77           | 0.31         | 19.3         |    |
| Flotation tailing           | 20.39           | 0.065        | 1.0          |    |
| Elutriated mica             | 3.84            | 2.34         | 0.1          |    |
| Slimes                      | 6.20            | 0.66         | 4.0          |    |
| Magnetic product            | 2.38            | 1.13         | 3.0          |    |
| Total head                  | 100.00          | 0.99         | 100.0        |    |
| Composite beryl concentrate | 6.54            | 9.6          | 63.6         |    |

Treatment of ore at intermediate sizes, by agglomeration tabling with only the minus 65-mesh ore ground through 100-mesh for flotation, resulted in a loss of only 4.0 percent of beryl in the slimes. Considerable beryl was lost in table rejects and only 63.6 percent of the BeO was recovered in a product assaying 9.6 percent BeO. The small loss of beryl in the slimes was offset by a large loss in the table rejects so that the greatest advantage of agglomeration tabling was the reduction in grinding cost made by treatment of ore at coarse sizes. Recovery could be raised and slime still kept at a minimum by grinding and floating beryl from the table rejects.

EXAMPLES NOS. 6, 7, AND 8.—MICA MOUNTAIN BERYL

Mica Mountain samples represent low-grade ores having an excess of mica and apatite, both of which should be removed to effectively concentrate the beryl. The following procedure was used for tests reported on both samples except that the higher grade sample was crushed through 48-mesh and the lower grade sample through 65-mesh.

1. The sample was roll crushed and screened on 20-mesh and 48-mesh screens. Clean mica rejected as plus 20-mesh material.

2. The mica was floated as previously described in the preceding examples, from the plus 48-mesh portion and the tailings were ground through 48-mesh and combined with original minus 48-mesh ore.

3. The minus 48-mesh ore was deslimed and selectively floated to remove mica, apatite, and beryl.

Final products were marketable mica and beryl concentrates and low-grade apatite products assaying 5 to 15 percent P<sub>2</sub>O<sub>5</sub>.

The two samples on which these three tests were made represent types of ore not amenable to concentration by any previously shown method. The higher grade sample, assaying 0.39 percent BeO, is the fine screen reject from a hand sorting operation. The lower grade sample, assaying only 0.17 percent BeO, is a mica schist with beryl dis-

tributed in small veinlets. Considering the extremely low grade of the samples and number of mineral separations made, results obtained are remarkably good.

Reagent consumptions and test results are tabulated in Tables 5 and 5A, 6 and 6A, and 7 and 7A.

TABLE 5.—REAGENT CONSUMPTION IN POUNDS PER TON OF ORE

|                     | H <sub>2</sub> SO <sub>4</sub> | NaF  | E. P. 487 | Oleic acid | X-1  | NaOH |
|---------------------|--------------------------------|------|-----------|------------|------|------|
| Mica flotation      | 15.60                          | 4.20 | 0.07      |            |      |      |
| Beryl rougher float | 0.92                           | 0.25 |           |            | 2.4  | 0.46 |
| Beryl cleaner float | 0.70                           | 0.25 |           |            | 0.9  | 0.02 |
| Apatite flotation   |                                |      |           |            | 0.08 | 1.7  |
| Total               | 17.22                          | 4.70 | 0.07      | 3.3        | 0.56 | 1.7  |

TABLE 5A

|                                 | Weight, percent | BeO, percent |              | 25 |
|---------------------------------|-----------------|--------------|--------------|----|
|                                 |                 | Assay        | Distribution |    |
| Beryl concentrate               | 2.78            | 10.5         | 77.8         |    |
| Mica product                    | 25.34           | 0.05         | 3.5          |    |
| Rougher flotation tailing       | 60.55           | 0.01         | 1.6          |    |
| Slimes                          | 6.38            | 0.44         | 7.4          |    |
| Apatite product                 | 2.20            | 0.49         | 2.9          |    |
| Beryl cleaner flotation tailing | 2.61            | 0.94         | 6.7          |    |
| Magnetic product                | 0.16            | 0.30         | 0.1          |    |
| Total head                      | 100.00          | 0.38         | 100.0        |    |

By flotation of minus 48-mesh ore, 77.8 percent of the BeO was concentrated in a product assaying 10.5 percent BeO. Separation of beryl and apatite was good. The apatite product assayed 15.05 percent P<sub>2</sub>O<sub>5</sub>.

TABLE 6.—REAGENT CONSUMPTION IN POUNDS PER TON OF ORE

|                   | H <sub>2</sub> SO <sub>4</sub> | NaF | E. P. 487 | Oleic acid | X-1  |
|-------------------|--------------------------------|-----|-----------|------------|------|
| Mica flotation    | 10.8                           | 2.6 | 3.2       |            |      |
| Beryl flotation   |                                | 3.2 |           | 0.4        | 0.08 |
| Apatite flotation |                                |     |           | 0.2        | 0.12 |
| Total             | 10.8                           | 5.8 | 3.2       | 0.6        | 0.20 |

TABLE 6A

|                           | Weight, percent | BeO, percent |              | 60 |
|---------------------------|-----------------|--------------|--------------|----|
|                           |                 | Assay        | Distribution |    |
| Mica concentrate          | 21.29           | .01          | 1.4          |    |
| Beryl concentrate         | 0.52            | 9.55         | 37.1         |    |
| Apatite product           | 4.36            | 0.18         | 1.9          |    |
| Cleaner flotation tailing | 0.60            | 0.29         | 1.5          |    |
| Rougher flotation tailing | 59.44           | 0.00         | 39.3         |    |
| Slimes                    | 13.59           | 0.16         | 14.8         |    |
| Magnetic product          | 0.20            | 0.03         | 0.0          |    |
| Total head                | 100.00          | 0.14         | 100.0        |    |

By flotation of minus 65-mesh ore, 37.1 percent of the BeO was concentrated in a product assaying 9.55 percent BeO. Oleic acid consumption was small and principal loss of beryl was in rougher flotation tailing. The beryl-apatite separation was good, apatite was floated before beryl with small reagent additions, and the apatite product without cleaning assayed 4.88 percent P<sub>2</sub>O<sub>5</sub> and only 0.18 percent BeO.

TABLE 7.—REAGENT CONSUMPTION IN POUNDS PER TON OF ORE

|                   | H <sub>2</sub> SO <sub>4</sub> | NaF   | E. P. 487 | Oleic acid | X-1  | NaOH |
|-------------------|--------------------------------|-------|-----------|------------|------|------|
| Mica flotation    | 11.2                           | 2.4   | 1.3       |            |      |      |
| Beryl flotation   | 1.85                           | 0.24  | -----     | 1.0        | 0.28 |      |
| Apatite flotation | -----                          | ----- | -----     | 1.8        | 0.43 | 1.2  |
| Total             | 12.05                          | 2.64  | 1.3       | 2.8        | 0.66 | 1.2  |

TABLE 7A

|                                   | Weight, percent | BeO, percent |              |
|-----------------------------------|-----------------|--------------|--------------|
|                                   |                 | Assay        | Distribution |
| Beryl-apatite product             | 1.3             | 4.30         | 40.9         |
| Beryl concentrate                 | 0.5             | 9.30         | 34.9         |
| Apatite cleaner flotation tailing | 2.6             | .280         | 5.2          |
| Beryl cleaner flotation tailing   | 3.2             | .170         | 3.8          |
| Rougher flotation tailing         | 55.2            | .010         | 4.5          |
| Mica concentrate                  | 28.1            | .018         | 3.8          |
| Slimes                            | 8.1             | .105         | 6.8          |
| Total head                        | 100.0           | .132         | 100.0        |

By flotation of minus 65-mesh ore 75.8 percent of the BeO was concentrated in two products, a beryl concentrate assaying 9.30 percent BeO and a beryl-apatite product assaying 4.30 percent BeO and 13.20 percent P<sub>2</sub>O<sub>5</sub>. Rougher beryl flotation

No amine was used in this test. The plus 100-mesh tailing, as a result, shows a high loss of beryl; 16.9 percent of the total BeO or 40.4 percent of the BeO in the coarse size.

#### EXAMPLE 10.—WISDOM BERYL

##### CLASS.—BERYL-PEGMATITE

The ore was stage ground in an iron ball mill to pass through a 48-mesh screen. The pulp was deslimed, braided iron was removed magnetically, and the sands were screened on 100-mesh into two sizes. Each size was conditioned and floated separately. In conditioning the coarse size, 0.22 pound of lauryl amine hydrochloride (E. P. 487) was added to activate the beryl. The pulp was filtered and the beryl floated with oleic acid. The concentrate was freed of garnets on a dry magnetic separator.

##### Reagents, pounds per ton of ore

|                     | Amine E. P. 487 | NaF  | H <sub>2</sub> SO <sub>4</sub> | Oleic acid | Emulsol X-1 | pH   |
|---------------------|-----------------|------|--------------------------------|------------|-------------|------|
| +100-mesh cond.     | 0.22            | 3.3  | 8.1                            | -----      | -----       | 2.3  |
| +100-mesh flotation | -----           | 0.11 | 0.2                            | 1.94       | 0.2         | 6.5  |
| -100-mesh cond.     | 2.2             | 10.1 | -----                          | -----      | -----       | 2.26 |
| -100-mesh flotation | 0.11            | 0.2  | 0.75                           | 0.15       | 0.15        | -6.7 |

##### Metallurgical data

| Product               | Assay No. | Grams, wt. | Percent, wt. | Assay, percent BeO | Units BeO | Distribution, percent BeO |
|-----------------------|-----------|------------|--------------|--------------------|-----------|---------------------------|
| Tailing +100-mesh     | 16369     | 308.0      | 36.01        | 0.05               | 0.015     | 1.6                       |
| Tailing -100-mesh     | 16370     | 302.0      | 35.30        | 0.015              | .005      | 0.5                       |
| Slimes                | 16371     | 142.0      | 16.60        | 0.74               | .123      | 13.0                      |
| Beryl conc. +100-mesh | Comp.     | 57.8       | 6.70         | 6.22               | .417      | 44.1                      |
| Beryl conc. -100-mesh | Comp.     | 46.1       | 5.39         | 7.17               | .387      | 40.8                      |
| Calc. head            |           | 855.4      | 100.00       | 0.95               | .947      | 100.0                     |

was satisfactory; the tailing made contained only 4.5 percent of the BeO as compared to 39.3 percent in the previous test.

#### EXAMPLE NO. 9.—WISDOM BERYL

##### CLASS.—BERYL-PEGMATITE

The ore was stage ground in an iron ball mill to pass through a 48-mesh screen. The pulp was deslimed, braided iron removed magnetically, and the sands were screened on 100-mesh into two sizes. Each size was conditioned, filtered, and floated separately.

##### Reagents, pounds per ton of ore

|                        | NaF  | H <sub>2</sub> SO <sub>4</sub> | Oleic acid | Emulsol X-1 | pH  |
|------------------------|------|--------------------------------|------------|-------------|-----|
| +100-mesh conditioning | 3.0  | 7.35                           | 3.5        | 0.7         | 2.3 |
| +100-mesh flotation    | 2.2  | 10.1                           | -----      | -----       | 6.7 |
| -100-mesh flotation    | 0.11 | 0.2                            | 0.75       | 0.15        | 6.8 |

##### Metallurgical data

| Product               | Assay No. | Grams, wt. | Percent, wt. | Assay, percent BeO | Units BeO | Distribution, percent BeO |
|-----------------------|-----------|------------|--------------|--------------------|-----------|---------------------------|
| Tailing +100-mesh     | 15722     | 330.0      | 34.70        | 0.45               | 0.160     | 16.9                      |
| Tailing -100-mesh     | 16370     | 371.0      | 37.95        | 0.615              | .006      | 0.6                       |
| Slimes                | 16371     | 174.4      | 17.85        | 0.74               | .123      | 12.9                      |
| Beryl conc. +100-mesh | Comp.     | 36.0       | 3.68         | 6.41               | .286      | 24.9                      |
| Beryl conc. -100-mesh | Comp.     | 55.6       | 5.79         | 7.17               | .415      | 42.7                      |
| Calculated head       |           | 977.0      | 100.00       | 0.95               | .949      | 100.0                     |

covered along with beryl and other beryllium minerals which largely increases the recovery of the beneficiation process.

Various changes can be made in the invention as illustrated and described since many apparently widely differing embodiments will occur to one skilled in the art.

What is claimed is:

1. In a process for the production of a beryllium ore concentrate, the improvement which comprises subjecting such an ore to a pretreatment to remove iron and then to a mineral-concentrating treatment involving selective filming under acidic conditions of a desired constituent in the presence of a soluble fluoride, a long-chain fatty acid and a long-chain alkyl amine salt.

2. In a process for the production of a beryllium ore concentrate, the improvement which comprises removing iron from such an ore, desliming said ore, then agitating and aerating the low-iron comminuted ore in an aqueous pulp at pH 2 to pH 6 in the presence of per ton of ore, from 0.2 to 10 pounds of a soluble fluoride, from 0.2 to 10 pounds of a long-chain fatty acid, and from 0.1 to 5.0 pounds of commercial long-chain alkyl amine salt.

3. In a process for the production of a beryllium ore concentrate, the improvement which comprises treating such a comminuted ore with a soluble fluoride and a strong mineral acid in an aqueous pulp, then washing the treated sands with excess water, and thereafter agitating and aerating an aqueous pulp of the thus-treated ore in the presence of a soluble fluoride, a strong mineral acid, oleic acid, and a mixture of long-chain alkyl amine salts corresponding to the coconut oil fatty acids.

4. In a process for the production of a beryllium ore concentrate, the improvement which comprises treating such a comminuted ore with a soluble fluoride, a strong mineral acid, and a long-chain alkyl amine salt in an aqueous pulp, then washing the treated sands with excess water, and thereafter agitating and aerating an aqueous pulp of the thus treated ore in the presence of a soluble fluoride, a strong mineral acid, and oleic acid.

HAROLD L. GIBBS.  
HENRY D. SNEDDEN.

### Certificate of Correction

Patent No. 2,395,475.

HAROLD L. GIBBS ET AL.

February 26, 1946.

It is hereby certified that errors appear in the printed specification of the above numbered patent requiring correction as follows: Page 5, first column, line 71, for the word "shown" read *known*; and second column, line 65, Table 6A, first column thereof, for "Total lead" read *Total head*; and that the said Letters Patent should be read with these corrections therein that the same may conform to the record of the case in the Patent Office.

Signed and sealed this 30th day of April, A. D. 1946.

[SEAL]

LESLIE FRAZER,  
First Assistant Commissioner of Patents.

covered along with beryl and other beryllium minerals which largely increases the recovery of the beneficiation process.

Various changes can be made in the invention as illustrated and described since many apparently widely differing embodiments will occur to one skilled in the art.

What is claimed is:

1. In a process for the production of a beryllium ore concentrate, the improvement which comprises subjecting such an ore to a pretreatment to remove iron and then to a mineral-concentrating treatment involving selective filming under acidic conditions of a desired constituent in the presence of a soluble fluoride, a long-chain fatty acid and a long-chain alkyl amine salt.

2. In a process for the production of a beryllium ore concentrate, the improvement which comprises removing iron from such an ore, desliming said ore, then agitating and aerating the low-iron comminuted ore in an aqueous pulp at pH 2 to pH 6 in the presence of per ton of ore, from 0.2 to 10 pounds of a soluble fluoride, from 0.2 to 10 pounds of a long-chain fatty acid, and from 0.1 to 5.0 pounds of commercial long-chain alkyl amine salt.

3. In a process for the production of a beryllium ore concentrate, the improvement which comprises treating such a comminuted ore with a soluble fluoride and a strong mineral acid in an aqueous pulp, then washing the treated sands with excess water, and thereafter agitating and aerating an aqueous pulp of the thus-treated ore in the presence of a soluble fluoride, a strong mineral acid, oleic acid, and a mixture of long-chain alkyl amine salts corresponding to the coconut oil fatty acids.

4. In a process for the production of a beryllium ore concentrate, the improvement which comprises treating such a comminuted ore with a soluble fluoride, a strong mineral acid, and a long-chain alkyl amine salt in an aqueous pulp, then washing the treated sands with excess water, and thereafter agitating and aerating an aqueous pulp of the thus treated ore in the presence of a soluble fluoride, a strong mineral acid, and oleic acid.

HAROLD L. GIBBS.  
HENRY D. SNEDDEN.

### Certificate of Correction

Patent No. 2,395,475.

HAROLD L. GIBBS ET AL.

February 26, 1946.

It is hereby certified that errors appear in the printed specification of the above numbered patent requiring correction as follows: Page 5, first column, line 71, for the word "shown" read *known*; and second column, line 65, Table 6A, first column thereof, for "Total lead" read *Total head*; and that the said Letters Patent should be read with these corrections therein that the same may conform to the record of the case in the Patent Office.

Signed and sealed this 30th day of April, A. D. 1946.

[SEAL]

LESLIE FRAZER,  
First Assistant Commissioner of Patents.